

April 21, 1925.

1,534,676

G. E. ANDREW

MANUFACTURE OF TAPE, CORD, YARN, ROPE, FABRIC, OR OTHER  
MATERIAL PRODUCED FROM FIBERS

Filed July 5, 1923

2 Sheets-Sheet 1



April 21, 1925.

1,534,676

G. E. ANDREW

MANUFACTURE OF TAPE, CORD, YARN, ROPE, FABRIC, OR OTHER  
MATERIAL PRODUCED FROM FIBERS

Filed July 5, 1923

2 Sheets-Sheet 2



Inventor  
G. E. Andrew  
By Marks & Clark  
Atteys.

Patented Apr. 21, 1925.

1,534,676

# UNITED STATES PATENT OFFICE.

GEORGE EDWARD ANDREW, OF NORTHWOOD, ENGLAND, ASSIGNOR TO F. P. LIMITED,  
OF JERSEY, CHANNEL ISLANDS.

MANUFACTURE OF TAPE, CORD, YARN, ROPE, FABRIC, OR OTHER MATERIAL PRO-  
DUCED FROM FIBERS.

Application filed July 5, 1923. Serial No. 649,692.

*To all whom it may concern:*

Be it known that I, GEORGE EDWARD ANDREW, C. B., a subject of the King of Great Britain and Ireland, and residing at 130 Green Lane, Northwood, in the county of Middlesex, England, have invented certain new and useful Improvements in the Manufacture of Tape, Cord, Yarn, Rope, Fabric, or other Material Produced from Fibers, of which the following is a specification.

This invention relates to the manufacture of tape, yarn, cord, rope, fabric or other material (hereinafter generically referred to as material) produced from fibers, and has particular reference to methods in which spun or unspun fibers and silk, cotton and other prepared yarns are employed for such manufacture.

The object of the present invention is to improve upon the hitherto known methods of the above kind and a particular advantage of the invention is that by its means it may be possible to employ fibers and the like hitherto thought to be unsuitable for the purpose while at the same time ensuring the utilization of the full strength of the fibers and the like and obtaining also complete protection from the harmful deleterious effects of moisture on the materials employed so that even those peculiarly subject to such harmful effects may be usefully adopted.

The invention consists in a method of forming tape, yarn, cord, rope, fabric or other material which comprises coating or impregnating fibers or yarns with vulcanized rubber latex.

The invention also consists in a method of forming tape, yarn, cord, rope or other fabric or material from unspun fibers by comprises the treatment of unspun fibers by means of vulcanized rubber latex in order to bind or cohere the fibers together to form a strip or band of determined width but of either undetermined or determined length.

The strip may be spun or twisted to form yarn, cord or the like and such yarns or the like may also be twisted or spun together to form larger cords, rope or the like.

Furthermore, the strips may be employed to form fabric of any length, width and thickness, and generally the invention may be adopted in the manufacture of any article or material hitherto formed from or suitable for formation from fibers.

The invention also consists in other details and arrangements hereinafter described or indicated.

In carrying my invention into effect in one convenient manner, I take unspun fibers of any suitable character and I may arrange these in the usual slivers and subject the same to any combing or like treatment whereby the fibers may be spread into a band of suitable dimensions determined by the size of strip required. Such fibers are then caused to pass through a bath of hot water or otherwise as may be required for subsequent treatment with ammonia or like suitable material acting as an anti-coagulant and/or preservative of latex, after which the fibers are passed through a bath of vulcanized rubber latex, being fed therethrough by rollers or other suitable means and any necessary or desired appurtenances or accessories may be provided for the purpose of expressing any surplus latex from the strip which issues from the bath. The strip is thereupon dried by suitable means and if it is to be formed into fabric a number of such strips may be arranged with the fibers all in one direction or with the fibers laid in various directions. For the formation of yarns or the like the strip is also dried and prior to twisting or spinning is preferably moistened with water. In such case I may employ a separating device to ensure that the yarn, cord or the like when spun shall be of the desired "count" or weight of fiber. In any modification of the invention the strip is preferably formed in known manner of a thickness approximating to the thickness of a single fiber, but this is not essential although it is preferably, as in this way each individual fiber becomes encased in its own envelope of latex.

In carrying my invention into effect in another convenient manner as, for example, in its application to silk, cotton or other prepared yarn, I cause the yarn to pass through a bath of hot water or otherwise as may be suitable for a subsequent treatment with ammonia or like suitable material acting as an anti-coagulant and/or preservative of latex, after which the yarn is passed through a bath of vulcanized rubber latex, being fed therethrough by rollers or other suitable means and any necessary or desired appurtenances or accessories may

be provided for the purpose of expressing any surplus latex from the yarn which issues from the bath and/or for imparting a smooth finish to the yarn. The yarn is 5 thereupon dried by suitable means.

For the formation of cords or the like by spinning a number of such prepared yarns the latter are preferably moistened with water.

- 10 The passing of the fiber, or prepared yarn, cord or the like through hot water, together with subsequent treatment with ammonia or like suitable material acting as an anti-coagulant, is essential for ensuring complete 15 impregnation with rubber in the form of an aqueous solution or colloidal suspension of rubber in water, and where it is important that as nearly as possible each fiber should be encased in the latex, it will be obvious 20 that very small amounts should be individually treated, but otherwise larger yarns may be so treated as, for example, when preparing ropes by a method in accordance with the invention.
- 25 I may employ latex vulcanized according to British patent application No. 193451 of 1921, the commercial advantages of the use of which include obviating the necessity of vulcanizing after application of the latex 30 to the fibers, yarn, cord, rope or the like, thereby eliminating the attendant disadvantages to the fibers or the like consequent upon exposing same to the deleterious effects of vulcanization, the articles so produced 35 are mechanically greatly superior in resilience and breaking strain, thermal qualities are much better and the commercial cost of production of the finished articles lower.

The accompanying drawings illustrate 40 several convenient forms of apparatus in accordance with the invention and in the construction of which I may use such substances, metals or the like suitable materials that no injurious or other chemical action 45 may arise during the process of preparation and impregnation with latex in a preserved condition in accordance with the invention. The baths, rollers, expressors or doctors and other machine parts which may 50 come into contact with the prepared liquids or solutions, also latex, may preferably be made from hard wood, ebonite or other similar substance, earthenware, slate, glass or other like material not readily affected by 55 chemical or other injurious action in order to avoid deleterious "after effects" upon the finished products.

Figure 1 is a diagrammatic side elevation 60 of one form of apparatus in accordance with the invention;

Figure 2 is a diagrammatic side elevation 65 of a portion of an alternative apparatus I may use in accordance with the invention for applying latex to yarns; cords or the like by "contact" impregnation, in combination

70 with a method I may use for maintaining the latex in mechanical mixture or solution with any contained dressing, drugs, loading matter or the like as may be required for the finished product;

Figure 3 shows sectional elevations of one 75 convenient form of controlled speed residue doffer;

Figures 4 and 5 are diagrammatic elevations of convenient forms of expressors or 80 doctors which I may use for removing surplus latex;

Figure 6 is a diagrammatic side elevation 85 of an alternative form of apparatus, and

Figures 7 and 8 are front views on a 90 larger scale of parts of Figure 6.

In the form of apparatus shown in Figures 1 to 5 the material to be treated is taken from the usual form of cop, spool, reel or bobbin, *a*, and led through a suitable tension control device, *b*, to a hot water bath, *c*, through which it passes submerged under suitable rollers, *d*, *d*', and before passing to the dilute alkali bath, *e*, it is caused to pass through a wringing device, *d*, comprising a suitable roller adapted for the material under preparation by the action of which any surplus water or the like resulting from the process is removed before the material passes to the dilute alkali or the 95 anti-coagulant bath, *e*, where it is caused to be partially submerged or totally submerged throughout the length of the bath as may be required by passing under or over rollers *e*', *e*', to ensure satisfactory preparation 100 for complete impregnation to result. The prepared material then passes to the latex bath, *g*, where it may be submerged or alternatively passed over latex roller *f*, for contact impregnation.

The latex bath is so constructed that a 105 minimum quantity of latex will suffice for continuous working; also I may provide a suitable device for causing the continued necessary fluid agitation when it is important to maintain a mechanical mixture in a suitable desired condition, which obtains when the latex is used with an admixture of dressing, drugs, loading matter or the like. The agitating device, *w*, (Figure 2) 110 comprises a submerged flow duct, together with suitable deflecting arrangements, which become operative in consequence of the fluid flow brought about by the partially immersed impregnating roller, *f*, and arranged 115 as illustrated.

The impregnated material on leaving the latex bath is taken to a series of rollers, two 120 of which are indicated, *j* and *l*, round which the material is caused to pass in different planes, the number of such rollers being dependent upon the size and nature of the material under operation for the purpose of mechanically assisting complete internal fiber impregnation.

- Any surplus latex which may be carried by the material is now removed by suitable expressors or doctors, convenient forms being indicated at Figures 4 and 5; these devices, *k* and *k'*, may be so arranged that the material shall pass freely the points of contact arranged for removal of surplus latex and so impart a smooth finish to the finished product.
- 10 The impregnated material thereafter passes in a suitable manner into a drying-off chamber, *t*, to creels, or rotary devices, *m* and *n*, capable of rotation in the same direction but with the axis of one creel or rotary device, *n*, arranged to be capable of adjustment as may be desired with reference to the axis of the other creel or rotary device, *m*, in order that the material may be caused to follow a helical path many times around both creels or rotary devices as may be necessary or desirable for the "drying-off" operation to be satisfactorily completed before the impregnated material is taken to the winding engine, *q*, for spooling on a suitable spool, cop, reel, bobbin or the like, *o*, as may be required for the finished product.
- 15 The impregnated material is received by the creels or rotary devices, *m* and *n*, in a moist condition, which would cause a certain amount of residue to deposit at the points of contact when in the moist condition and to remove same in order to maintain the creels or rotary devices in a condition fit for continued use. I may employ a roller brush or other like suitable residue doffing device capable of being so employed and so adapted that its relative peripheral speed to that of the adjacent creel or rotary device may be under control.
- 20 I may use in accordance with the invention a convenient form of controlled speed residue doffer, *s*, as illustrated in Figure 3, comprising a suitable drum capable of rotation around a fixed bar or shaft, the axis of which is capable of adjustment relative to the adjacent creel or rotary device and provided with a fabric brush attachment along and around its external diameter and fitted with a helical spring friction control attachment, substantially as illustrated.
- 25 Figures 6 to 8 illustrate one convenient form of apparatus for separating the rubberized fiber strip which may be used in accordance with the invention for producing narrow widths of strip to the desired "count" as may be required. Figure 6 is a diagrammatic side elevation of the apparatus. Figure 7 is a diagrammatic section and elevation of the roller with separating face provided for securely holding in position the rubberized fiber strip when under process of separation into narrow widths to the desired "count" or fiber weight. Figure 8 is a diagrammatic section and elevation of one convenient method of forming a separating device, *y*, which comprises a series of thin circular knives, spaced suitably to desired width and which rapidly revolve, the lower portion being immersed in a cold water bath as indicated at *x*, Figure 6. 70 The roller, *v*, provided with separating face, is in this convenient arrangement free to revolve and does so by virtue of its being in close contact with the moving strip under process of separation, but I may arrange this roller to be operated by suitable mechanism connected with the receiving drum, *z*. The direction of rotation of separating face roller, *v*, is conveniently arranged to be contrary to that of the separating device, *y*, and the speed of rotation of the separating device, *y*, is greater than that of the separating roller, *v*. In this convenient form of separating device the rubberized strip to be separated is arranged 75 to be taken from a suitable swift or strip holder, *h*, which is arranged to be capable of giving a controlled supply of strip as may be required, and it may be provided with a suitable friction delay device to ensure the strip being under control and taut, substantially as illustrated at *i*. The controlled strip on its way to the tension rollers or fixed bars, *p*, is required to pass a "correcting plane device," *r*, which comprises a perfectly smooth bar or series of bars or other similar mechanism, such as an adjustable angle plate or plates with a smooth edge or series of edges over which the strip may pass smoothly and which may be capable of adjustment to any convenient angle as may be necessary to maintain alignment and relative position of the moving strip to certain fixed positions on the separating face roller in order that the strip 80 may be delivered free from puckers, creases, doubling or the like and ensuring the separated strips being of the correct "count" or fiber weight. The strip then passes from the tension rollers or bars, *p*, under and 85 round rollers, *v* and *u*, as indicated in Figure 6, both of these rollers being free to revolve at the same peripheral speed as that of the strip under process of separation. The rubberized strip is securely held in position against the separating face of roller, *v*, by virtue of its being under suitable tension between the points of its contact with tension rollers, *p*, and *p'*. The rapidly revolving separating device, *y*, operates 90 against the direction of motion of the strip under process of separation and the speed of rotation of same is arranged to be relatively much greater than that of the separating face roller and in this convenient 95 form of apparatus I arrange for the separating device to be operated at the required speed by a suitable independent drive. The separated narrow strips are now passed 100 over, under or around one or more of the 105
- 110
- 115
- 120
- 125
- 130

tension rollers,  $p'$ , as may be necessary to ensure an even winding on the receiving drum,  $z$ , which may be arranged to be operated by either hand or power as required. The rollers  $u$  and  $v$  are so arranged as to be capable of concurrent vertical axial adjustment relative to separating device,  $y$ , as illustrated. I may provide a suitable bath of cold water,  $w$ , in which the separating device may be partially immersed or, alternatively, I may provide a suitable cold water spray for the separating device when in use in order to ensure a perfectly clean and even separation into narrow widths of strip and also to maintain the separating device in a condition suitable for continued operation.

The invention is not to be limited to the details hereinbefore given by way of illustration, and the precise methods adopted in the manufacture and the means employed for carrying such methods into effect may be suitably modified depending upon any particular practical requirements that may have to be fulfilled.

Claims:

1. A method of forming material from fibers which comprises passing the fibers through an anti-coagulant for latex and then through vulcanized rubber latex prior to further treatment for the formation of the material.

2. A method of forming material from fibers which comprises passing the fibers through a bath of ammonia and then through vulcanized rubber latex prior to further treatment for the formation of the material.

3. A method of forming material from fibers which comprises passing the fibers

through hot water, then through an anti-coagulant for latex and finally through vulcanized rubber latex prior to further treatment for the formation of the material.

4. A method of forming material from fibers which comprises passing the fibers through hot water then through ammonia and finally through vulcanized rubber latex prior to further treatment for the formation of the material.

5. A method of forming material from fibers which comprises forming the fibers into yarn passing the yarn through an anti-coagulant for latex and then through vulcanized rubber latex prior to further treatment for the formation of the material.

6. A method of forming material from fibers which comprises forming the fibers into yarn, passing the yarn through hot water then through an anti-coagulant for latex and finally through vulcanized rubber latex prior to the further treatment of the yarn for the formation of the material.

7. A method of forming material from fibers which comprises spreading the fibers to form a strip of a thickness approximating to the thickness of a single fiber passing said fiber strip through an anti-coagulant for latex and then through vulcanized rubber latex prior to further treatment to form the finished material.

8. A method of forming material from fibers which comprise passing a fiber yarn through a bath of hot water, then through an anti-coagulant for latex and finally through vulcanized rubber latex.

In testimony whereof I have signed my name to this specification.

GEORGE EDWARD ANDREW.